# EUROPEAN PATENT APPLICATION

(11) **EP 0 397 086 A2**
(43) Date of publication of application: **14.11.1990**
(21) Application number: 90108586.0
(22) Date of filing: 07.05.1990
(51) Int. Cl.: G03C 7/30

(54) **A method for the manufacture of silver halide color photographic light sensitive materials**

(30) Priority: 10.05.1989 JP 116835/89
(71) Applicant: FUJI PHOTO FILM CO., LTD., Kanagawa (JP)
(72) Inventor: Fukuoka, Masahiro, c/o Fuji Photo Film Co., Ltd., Minami Ashigara-shi, Kanagawa (JP)
(74) Representative: Hansen, Bernd, Dr. Dipl.-Chem.

(57) **Abstract**

A method for manufacturing a silver halide color photographic light sensitive material comprising a support having thereon at least one of light sensitive silver halide emulsion layer and non-light sensitive hydrophilic colloid layer which contain at least one hydrophobic photographically useful additive, which comprises preparing a hydrophobic colloid emulsified dispersion of said hydrophobic photographically useful additive, mixing the emulsified dispersion within 24 hours with the remaining coating composition of the layer and coating the mixture obtained on the support.

## Description

### FIELD OF THE INVENTION

This invention concerns a method for the manufacture of silver halide color photographic light sensitive materials.

### BACKGROUND OF THE INVENTION

Silver halide color photographic light sensitive materials are generally manufactured by coating at least one light sensitive silver halide emulsion layer which contains hydrophobic additives, such as couplers, and non-light sensitive hydrophilic colloid layers which contain hydrophobic photographically useful additives, such as ultraviolet absorbers, onto a support.

In the past, the manufacture of color light sensitive materials has involved first preparing a hydrophilic colloid dispersions which contains a hydrophobic photographically useful additive and then, storing it for from 3 to 100 days at a temperature about 27°C or below, remelting as small lots, mixing it with the remainder of the coating liquid, such as the silver halide emulsion, to form a coating liquid for a photographic layer of the type mentioned above, and coating it onto a support.

With the sensitive materials for color printing purposes (color papers) which have a reflective support from among the latest color sensitive materials, there has been an increasing demand for a high maximum color density (Dmax) and excellent stability (fastness) of the colored image with the passage of time after color development processing in particular, and the inventors have made a detailed study of the aging of hydrophobic colloid dispersions which contain hydrophobic photographically useful additives and the resulting effects on photographic performance and coated surface quality.

As a result it has been discovered that by mixing the hydrophilic colloid emulsified dispersions containing a hydrophobic coupler with a silver halide emulsion without delay after prepared, not only a high Dmax (high contrast) is obtained, but the fastness of the colored image after color development processing is also improved, and there is no problem in respect of the coated surface quality. Furthermore, it has been discovered that staining is prevented and that there are no problems with the coated surface quality when, after preparing a hydrophilic colloid emulsified dispersion containing hydrophobic ultraviolet absorbers and/or anti-color mixing agents, for example, the emulsified dispersion is mixed without delay with the remainder of the coating liquid (aqueous gelatin solution) to form a non-light sensitive layer coating liquid and is coated. The present invention is based upon such findings.

In the past, the mixing of an oil in water type dispersion of certain types of coupler and a silver halide emulsion immediately before coating and the coating of the coating liquid onto the support was suggested in JP-A-63-296046, JP-A-63-296038 and JP-A-61-90154 for preventing the coating irregularities and loss of photographic speed for example which arise when the coupler dispersion and the silver halide emulsion are mixed together and left to stand before coating, but the effect on photographic performance and the coated surface quality due to aging after preparing the hydrophilic colloid dispersion which contains the hydrophobic photographically useful additives is not fully elucidated. (The term "JP-A" as used herein signifies an "unexamined published Japanese patent application".)

### SUMMARY OF THE INVENTION

The first object of the present invention is to provide a method for manufacturing a silver halide color photographic light sensitive materials which provide a high Dmax (high contrast), and which provide colored images which have excellent fastness after color development processing and with which, moreover, the coated surface quality is good.

The second object of the present invention is to provide a method for manufacturing silver halide color photosensitive materials in which problems with the coated surface quality and with the change in photographic performance due to aging after preparing the coating liquids are slight.

The objects of the present invention can be attained effectively by the method indicated below.
1) A method for manufacturing a silver halide color photographic light sensitive material comprising a support having thereon at least one of a light sensitive silver halide emulsion layer and a non-light sensitive hydrophilic colloid layer which contains at least one hydrophobic photographically useful additive, which comprises preparing a hydrophobic colloid emulsified dispersion of the hydrophobic photographically useful additive, mixing the emulsified dispersion within 24 hours with the remaining coating composition of the layer, and coating the mixture obtained.
2) A method for manufacturing a silver halide color photographic light sensitive materials as described in (1) wherein the mixture of the hydrophilic colloid emulsified dispersion and the remaining coating composition of the layer is coated within three hours after mixing.

### DETAILED DESCRIPTION OF THE INVENTION

The invention is described in detail below.

In the present invention, mixing the hydrophilic colloid emulsified dispersion (hereinafter referred to hydrophilic colloid dispersion) with the remaining coating composition is conducted within 24 hours, preferably within 12 hours, more desirably within 6 hours and most desirably within 3 hours afater preparing the hydrophilic colloid dispersion of the hydrophobic photographically useful additives (hereinafter referred to hydrophobic additives). The standing time is preferable as short as possible. The temperature of the hydrophilic colloid dispersion during the standing time is preferably from about 6°C to 70°C, and most desirably from about 6°C to 50°C.

In the present invention the coating of thus prepared mixture is generally conducted within 3 hours, preferably within 2 hours, more preferably within one hour and most preferably within 30 minutes. The standing time is preferably as short as possible that it may be 5 minutes or less. Furthermore, the temperature of the mixture during the standing time is preferably from about 30°C to 60°C, and more desirably from about 35°C to 50°C.

In the present invention the hydrophobic colloid emulsified dispersion of at least one hydrophobic additive can be obtained by a conventional method which is used in preparation of silver halide color photographic materials. Usually, the dispersion is prepared as follows.

As a dispersion medium a hydrophilic colloidal aqueous solution is used. As a hydrophilic colloid, gelatin is advantageously used but other hydrophilic colloids can also be used alone or together with gelatin. Any gelatin can be used in the present invention. Examples of gelatin include lime-treated gelatin and acid-treated gelatin with lime-treated gelatin being preferrred. The concentration of gelatin in the colloidal aqueous solution is preferably of from 10 to 50 weight%, more preferably 20 to 40 weight%. When the concentration is less than 10 weight%, recrystalization or troubles with respect to the coated surface quality tends to occur, on the other hand, when the concentration exceeds 50 weight%, drops having undesirably large size tend to form or troubles with respect to the coated surface quality tend to occur. The hydrophilic colloidal aqueous solution usually contains a surfactant as an emulsifying agent.

Examples of the hydrophobic photographically useful additives include couplers, anti-color mixing agents, antifoggants, anti-color fading agents, anti-staining agents, ultraviolet absorbers, and slidability improving agents.

These additives are dispersed into a hydrophilic colloid aqueous solution as an organic solvent solution thereof. Usually, the concentration of the additive in a solvent is from 50 to 150 weight%, based on the weight of the solvent.

As organic solvents those which has a high boiling point (described hereinafter in detail) can be used alone or in combination with an organic solvent having a low boiling point, such as alcohol and acetone. When the additive is soluble to the organic solvent having a low boiling point, the additive may be added to a colloidal solution as a solution of such an organic solvent. This solvent is removed by evaporation prior to the mixing in the same manner as in conventional methods for preparation of silver halide photographic materials. The high boiling point organic solvent is usually used in an amount of from 0 weight% (in the case when a low boiling point organic solvent is used alone) to 10 weight% based on the total weight of the dispersion.

The remaining coating composition which is mixed with the hydrophilic colloid dispersion of the hydrophobic additives is typically a silver halide emulsion in the case for coating a light sensitive silver halide emulsion layer, and in the case for coating a non-light sensitive layer it is typically an aqueous colloidal solution. As the aqueous colloidal solution the same solution as described for the dispersion medium for the hydrophobic additives can be used.

In the present invention, the remaining coating composition preferably does not contain any hydrophobic additive, especially, the silver halide emulsion (as the remaining coating composition) preferably does not contain any hydrophobic additive.

Photographically useful additives other than the hydrophobic additives can be incorporated either to the hydrophilic colloid dispersion or to the remaining coating composition.

In the silver halide emulsion usually a sensitizing dye is incorporated.

Examples of the non-light sensitive layer is a protective layer, an antihalation layer, and an inter- mediate layer (such as an ultraviolet absorbing layer, an anti-color mixing layer and an anti-irradiation layer). An ultraviolet absorber is usually contained in the non-light sensitive layer, and a slidability improving agent is contained in a protective layer.

The amount of the hydrophilic colloid emulsified dispersion is usually from about 1 to 70 weight% based on the total weight of the coating composition obtained by mixing the dispersion with the remained coating composition.

When the hydrophobic additive is a liquid paraffin which is used as a slidability improving agent the amount is preferably about 1 to 10 weight%, and when the hydrophobic additive is a coupler, an anti-color mixing agent, an antifoggant, an anti-color fading agent, an anti-staining agent or an ultraviolet absorber, the amount is preferably from about 10 to 60 weight%.

The average particle size of the hydrophobic additives in the coating liquid which are used in the present invention is preferably not more than 0.2 µm, more preferably not more than 0.15 µm, and most preferably not more than 0.1 µm. The size may be as small as, for example, about 0.01 µm.

The average particle size of the fine particle dispersions in such a coating liquid can be measured using the well known turbidity method or using apparatus such as the Nanosizer made by the British Coal Tar Co.

The method for the emulsification and dispersion of these additives is further described in detail hereinafter using couplers as a typical example.

The effect of the present invention is especially pronounced when applied to systems where cyan couplers are used among the couplers, and this is desirable.

Furthermore, the present invention is more effective in cases where dispersions of hydrophobic cyan, magenta and yellow couplers are used in systems in which high silver chloride-content emulsions (not less than 80 mol% of silver chloride) are used, and this is desirable.

The effects of the present invention is remarkable when the method of the present invention is applied to a system wherein a high silver chloride-content emulsion is used.

When a pyrazoloazole coupler is used as a hydrophobic additive, the silver halide emulsion may be either a system wherein a silver chlorobromide emulsion is used or a system wherein a high silver chloride- content emulsion is used, in order to obtain a high D max (high contrast).

Furthermore, the improving effect on the light fastness of the colored image is especially pronounced in systems where a high silver chloride-content emulsion is used and processing is carried out in an essentially benzyl alcohol free color development bath.

Here, the term "essentially benzyl alcohol free" signifies that there is not more than 2 ml of benzyl alcohol per liter of color development bath, and a pronounced fastness improving effect is obtained when the benzyl alcohol concentration is not more than 0.5 ml/ℓ, and especially when the color development bath contains no benzyl alcohol at all.

On the other hand, in connection with troubles of the coated surface, phenol based cyan couplers which have an acylamino group in the 2-position and a methyl group in the 5-position, and benzotriazole based ultraviolet absorbers which are solids at normal temperatures, for example, are liable to recrystallization in the hydrophilic colloid dispersion or in the coating liquid and they are liable to cause coating troubles, but this troubles can be prevented effectively by applying this present invention.

The above-mentioned effects of the present invention are especially pronounced in those cases where oil in water dispersions are used.

The embodiments relating to the method for production of color light sensitive materials in accordance with the present invention are described in detail below.

The color photographic light sensitive materials of this present invention can be formed by coating at least one blue sensitive silver halide emulsion layer, at least one green sensitive silver halide emulsion layer and at least one red sensitive silver halide emulsion layer on a support. Normally, these layers are coated on the support in the order indicated above for a general color printing paper, but different orders can be adopted. Furthermore, they may have a infrared sensitive silver halide emulsion layer in place of at least one of the aforementioned emulsion layers. Color reproduction can be achieved with these color light sensitive emulsion layers with the subtractive color method using silver halide emulsions which are sensitive to the different wavelength regions and couplers which forms dyes relating to the complementary color of the light to which the layers are sensitive, which is to say by including a color coupler which forms a yellow color in the blue sensitive layer, a color coupler which forms magenta in the green sensitive layer and a color coupler which forms cyan in the red sensitive layer. However, the structure may take a form which does not have the above-mentioned correspondence between the light sensitive layers and the hues formed by the couplers.

The use of essentially silver iodide free silver chlorobromide or silver chloride for the silver halide in the present invention is preferred. Here, the term "essentially silver iodide free" signifies that the silver iodide content is not more than 1 mol%, and preferably not more than 0.2 mol%. The halogen composition in the emulsion may differ from grain to grain or it may be uniform. The nature of the grains can easily be made homogeneous when emulsions which have a halogen composition which is the same from grain to grain are used. Furthermore, the halogen composition distribution within the grains of the silver halide emulsion may be such that the grains have a so-called uniform structure in which the composition is the same in all parts of the silver halide grain, or it may be such that the grains have a so-called laminated structure in which the core inside the silver halide grain has a different halogen composition from the shell (a single layer or a plurality of layers) which surrounds the core, or it may be such that the grains are of a structure which has parts which have a different halogen composition which are not in the form of a layer within the grains or at the grain surface (when present at the grain surface, the structure is such that the parts which have a different composition are jointed on the edge, corner, or plane of the grain) for example, and grains which have any such halogen composition distribution can be selected appropriately for use. The use of either of the latter two types of grain is preferable to the use of grains which have a uniform halogen composition for obtaining higher photographic speeds, and it is also preferred from the viewpoint of pressure resistance. In those cases where the silver halide grains have a structure as described above, the boundaries between the parts which have different halogen compositions may be distinct boundaries, or there may be an indistinct boundary with the formation of mixed crystals due to the difference in composition, or there may be a positive continuous variation in the structure.

The halogen composition of these silver chlorobromide emulsions can have any silver bromide/silver chloride ratio. This ratio can have a wide range, depending on the intended purpose, but the use of those which have a silver chloride content of at least 2 mol% are preferred.

Furthermore, the use of so-called high silver chloride-content emulsions which have a high silver chloride content is preferred in light sensitive materials which are suitable for rapid processing. The silver chloride content of these high silver chloride-content emulsions is preferably at least 90 mol%, and most desirably at least 95 mol%.

A structure which has a silver bromide local phase in the form of a layer or in some other form, as described above, within and/or at the surface of the silver halide grain is desirable for these high silver chloride-content emulsions. The halogen composition of the above-mentioned local phase preferably has a silver bromide content of at least 10 mol%, and most desirably it has a silver bromide content in excess of 20 mol%. This local phase can be present within the grain, or at the edge, corner, or plane of the grain, and in a preferred embodiment the local phase is grown epitaxially on the corner of the grain.

On the other hand, the use of grains which have a uniform type structure with a small halogen composition distribution within the grain is also desirable in high silver chloride-content emulsions which have a silver chloride content of at least 90 mol% for greatly suppressing the fall in sensitivity which occurs when pressure is applied to a photographic material.

Furthermore, increasing the silver chloride content of the silver halide emulsion is also effective for reducing the rate of replenishment of development processing baths. The use of an almost pure silver chloride emulsion such that the silver chloride content is from 98 mol% to 100 mol% is desirable in such cases.

The average grain size (where the grain size is taken to be the diameter of a circle which has an area equal to the projected area of the grain and the average grain size is taken to be the average of these values) of the silver halide grains which are included in the silver halide emulsions which are used in this present invention is preferably from 0.1 µ to 2 µ.

Furthermore, the size distribution of these grains is preferably a mono-dispersion of which the variation coefficient (the value obtained by dividing the standard deviation of the grain size distribution by the average grain size) is not more than 20%, and preferably not more than 15%. Blending of the above-mentioned mono-disperse emulsions in the same layer, or lamination coating of the above-mentioned mono-dispersions, is desirable for obtaining a wider latitude.

The form of the silver halide grains which are contained in a photographic emulsion may be a regular crystalline form, for example, a cubic, tetradecahedral or octahedral form, an irregular crystalline form, for example, a spherical or tabular form, or it may be a form which is a composite of these forms. Furthermore, the emulsion may also be comprised of grains which have various crystalline forms. In the present invention, the inclusion of at least 50%, preferably at least 70%, and most desirably at least 90%, of grains which have the above-mentioned regular crystalline forms is preferred.

Furthermore, the use of emulsions in which tabular grains of which the average aspect ratio (diameter of the calculated circle/thickness) is at least 5, and preferably at least 8, account for more than 50% of all the grains in terms of projected area is also desirable.

The silver chlorobromide emulsions used in the present invention can be prepared using the methods disclosed, for example, by P. Glafkides in Chimie et Physique Photographique, published by Paul Montel, 1967, by G.F. Duffin in Photographic Emulsion Chemistry, published by Focal Press, 1966, and by V.L. Zelikmann et al. in Making and Coating Photographic Emulsions, published by Focal Press, 1964. That is to say, they can be prepared using acidic.methods, neutral methods and ammonia methods for example, and a single jet method, a double jet method, or a combination of such methods, can be used for reacting the soluble silver salt with the soluble halide. Methods in which the grains are formed in the presence of an excess of silver ions (so-called reverse mixing methods) can also be used. The method in which the pAg value in the liquid phase in which the silver halide is being formed is held constant, which is to say the so-called controlled double jet method, can be used as one type of simultaneous mixing procedure. It is possible to obtain silver halide emulsions with a regular crystalline form and an almost uniform grain size in this method.

Various multi-valent metal ion impurities can be introduced into the silver halide emulsions which are used in the present invention during the formation or physical ripening of the emulsion grains. For example, salts of cadmium, zinc, lead, copper or thallium, or salts or complex salts of iron, ruthenium, rhodium, palladium, osmium, iridium and platinum, for example, which are group VIII elements in the Periodic Table, can be used as compounds of this type. The use of the above-mentioned group VIII elements is especially desirable. The amount of these compounds added varies over a wide range, depending on the intended purpose, but an amount of from 10⁻⁹ to 10⁻² mol per mol of silver halide is preferred.

The silver halide emulsions used in this present invention are normally subjected to chemical sensitization and spectral sensitization.

Sulfur sensitization which is typified by the addition of unstable sulfur compounds, precious metal sensitization which is typified by gold sensitization, and reduction sensitization, for example, can be used individually or conjointly as chemical sensitization methods. The use of the compounds disclosed from the lower right hand column on page 18 to the upper right and column on page 22 of JP-A-62-215272 for the compounds which are used for chemical sensitization is preferred.

Spectral sensitization is carried out with a view to rendering each emulsion layer in a photosensitive material of the present invention sensitive to light of the prescribed wavelength region. In the present invention, this is preferably achieved by adding dyes (spectrally sensitizing dyes) which absorb light in the wavelength regions corresponding to the necessary spectral sensitivity. Examples of spectrally sensitizing dyes which can be used are disclosed, for example, by F.M. Harmer in Heterocyclic Compounds, Cyanine Dyes and Related Compounds, (John Wiley & Sons [New York, London], 1964). Examples of actual preferred compounds which can be used have been disclosed from the upper right hand column on page 22 to page 38 of the specification JP-A-62-215272.

Various compounds or precursors thereof can be added to the silver halide emulsions which are used in the present invention with a view to preventing the occurrence of fogging or with a view to stabilizing photographic performance during the manufacture, storage or photographic processing of the photographic material. Actual examples of such compounds are disclosed on pages 39-72 of the aforementioned JP-A-62-215272, and the use of these compounds is preferred.

The emulsions used in the present invention may be of the so-called surface latent image type in which the latent image is formed principally on the grain surfaces, or of the so-called internal latent image type in which the latent image is formed principally within the grains.

Yellow couplers, magenta couplers and cyan couplers which form yellow, magenta and cyan colors respectively on coupling with the oxidized product of a primary aromatic amine color developing agent are normally used in color photographic materials of the present invention.

Use of cyan couplers, magenta couplers and yellow couplers which can be represented by the general formulae (C-I), (C-II), (M-I), (M-II) and (Y) which are indicated below is preferred in this present invention.

In general formulae (C-I) and (C-II), R₁, R₂ and R₄ each represents substituted or unsubstituted aliphatic, aromatic, or heterocyclic groups, R₃, R₅ and R₆ each represents hydrogen atoms, halogen atoms, aliphatic groups, aromatic groups or acylamino groups, and R₃ together with R₂ may represent a group of non-metal atoms which is required to form a 5- or 6-membered nitrogen containing ring. Y₁ and Y₂ each represents hydrogen atoms or groups which can be eliminated at the time of a coupling reaction with the oxidized product of a developing agent. Moreover, n represents 0 or 1.

R₅ in general formula (C-II) is preferably an aliphatic group, for example, methyl, ethyl, propyl, butyl, pentadecyl, tert-butyl, cyclohexyl, cyclohexylmethyl, phenylthiomethyl, dodecyloxyphenylthiomethyl, butanamidomethyl or methoxymethyl.

Preferred examples of the cyan couplers which can be represented by the aforementioned general formula (C-I) or (C-II) are described below.

R₁ in general formula (C-I) is preferably an aryl group or a heterocyclic group, and aryl groups substituted with halogen atoms, alkyl groups, alkoxy groups, aryloxy groups, acylamino groups, acyl groups, carbamoyl groups, sulfonamido groups, sulfamoyl groups, sulfonyl groups, oxycarbonyl groups and cyano groups are most desirable.

In those cases where R₃ and R₂ do not form a ring in general formula (C-I), R₂ is preferably a substituted or unsubstituted alkyl group or aryl group, and most desirably a substituted aryloxy substituted alkyl group, and R₃ is preferably a hydrogen atom.

R₄ in general formula (C-II) is preferably a substituted or unsubstituted alkyl group or aryl group, and most desirably a substituted aryloxy substituted alkyl group.

R₅ in general formula (C-II) is preferably an alkyl group which has from 2 to 15 carbon atoms or a methyl group which has a substituent group having at least 1 carbon atom, and the preferred substituent groups are arylthio groups, alkylthio groups, acylamino groups, aryloxy groups and alkyloxy groups.

R₅ in general formula (C-II) is most desirably an alkyl group which has from 2 to 15 carbon atoms, and alkyl groups which have from 2 to 4 carbon atoms are especially desirable.

R₆ in general formula (C-II) is preferably a hydrogen atom or a halogen atom, and most desirably it is a chlorine atom or a fluorine atom. Y₁ and Y₂ in general formulae (C-I) and (C-II) each preferably represent a hydrogen atom, a halogen atom, an alkoxy group, an aryloxy group, an acyloxy group or a sulfonamido group.

In general formula (M-I), R₇ and R₉ each represents aryl groups, R₈ represents a hydrogen atom, an aliphatic or aromatic acyl group, or an aliphatic or aromatic sulfonyl group, and Y₃ represents a hydrogen atom or a releasing group. The substituent groups permitted for the aryl groups (preferably phenyl groups) represented by R₇ and R₉ are the same as those permitted as substituent groups for R₁, and when there are two or more substituent groups these may be the same or different. R₈ is preferably a hydrogen atom, an aliphatic acyl group or sulfonyl group, and most desirably it is a hydrogen atom. Y₃ is preferably a group of the type which is eliminated at a sulfur, oxygen or nitrogen atom, and most desirably it is a sulfur atom releasing group of the type disclosed, for example, in U.S. Patent 4,351,897 or International Patent Publication WO88/04795.

In general formula (M-II), R₁₀ represents a hydrogen atom or a substituent group such as a halogen atom, an alkyl group, an aryl group, a heterocyclic group, a cyano group, an alkoxy group, an aryloxy group, a heterocyclyloxy group, an acyloxy group, a carbamoyloxy group, a silyloxy group, a sulfonyloxy group, an acylamino group, an anilino group, an ureido group, an imido group, a sulfamoylamino group, a carbamoylamino group, an alkylthio group, an arylthio group, a heterocyclylthio group, an alkoxycarbonylamino group, an aryloxycarbonylamino group, a sulfonamido group, a carbamoyl group[, an acyl group, a sulfamoyl group, a sulfonyl group, a sulfinyl group, an alkoxycarbonyl group, or an aryloxycarbonyl group. Y₄ represents a hydrogen atom or a releasing group such as a halogen atom, a carboxy group, or a coupling releasing group which is attached to the carbon atom located at the couling position through its oxygen, nitrogen or sulfur atom, and it is preferably a halogen atom or an arylthio group, Za, Zb and Zc each represents a methine group, a substituted methine group, =N- or -NH-, and one of the bonds Za-Zb and Zb-Zc is a double bond and the other is a single bond. Those cases where the Zb-Zc bond is a carbon-carbon double bond include cases in which this bond is part of an aromatic ring. Cases where a dimer or larger oligomer is formed via R₁₀ or Y₄, and cases in which, when Za, Zb or Zc is a substituted methine group, a dimer or larger oligomer is formed via the substituted methine groups, are included.

Among the pyrazoloazole based couplers represented by general formula (M-II), the imidazo[1,2-b]pyrazoles disclosed in U.S. Patent 4,500,630 are preferred from the point of view of the slight yellow side absorbance and the light fastness of the colored dye, and the pyrazolo-[1,5-b][1,2,4]triazole disclosed in U.S. Patent 4,540,654 is especially desirable.

The use of the pyrazolotriazole couplers in which a branched alkyl group is bonded directly to the 2-, 3- or 6-position of the pyrazolotriazole ring as disclosed in JP-A-61-65245, the pyrazoloazole couplers which have a sulfonamido group within the molecule as disclosed in JP-A-61-65246, the pyrazoloazole couplers which have alkoxyphenylsulfonamido ballast groups as disclosed in JP-A-61-147254, and the pyrazolotriazole couplers which have an alkoxy group or an aryloxy group in the 6-position as disclosed in European Patents (laid open) 226,849 and 294,785 is also desirable.

In general formula (Y), R₁₁ represents a halogen atom, an alkoxy group, a trifluoromethyl group or an aryl group, and R₁₂ represents a hydrogen atom, a halogen atom or an alkoxy group. A represents -NHCOR₁₃, -NHSO₂- R₁₃, -SO₂NHR₁₃, -COOR₁₃ or where R₁₃ and R₁₄ each represents an alkyl, an aryl group or an acyl group. Y₅ represents a releasing group. The substituent groups for R₁₂, R₁₃ and R₁₄ are the same as the substituent groups permitted for R₁, and the releasing group Y₅ is preferably a group of the type with which elimination occurs at an oxygen atom or a nitrogen atom, and it is most desirably of the nitrogen atom releasing type.

Actual examples of couplers which can be represented by general formulae (C-I), (C-II), (M-I), (M-II) and (Y) are indicated below.

The couplers represented by the above-mentioned general formulae (C-I) to (Y) are normally include in the silver halide emulsion layers which form the light sensitive layer in an amount of from 0.1 to 1.0 mol, and preferably of from 0.1 to 0.5 mol, per mol of silver halide.

Various known techniques can be used in the present invention for the emulsification and dispersion of the aforementioned couplers in hydrophilic colloids. Normally, they can be added by means of oil in water dispersion method using the oil protection method where, after being dissolved in a solvent, the solution is emulsified and dispersed in an aqueous gelatin solution which contains a surfactant. Alternatively, water or an aqueous gelatin solution can be added to a coupler solution which contains a surfactant to form oil in water dispersion by phase reversal. The coupler dispersion can be mixed with photographic emulsion after removing low boiling point organic solvents by distillation, noodle washing or ultrafiltration for example.

The use of high boiling point organic solvents which have a dielectric constant (25°C) of from 2 to 20 and a refractive index (25°C) of from 1.5 to 1.7, and/or water insoluble polymeric compounds, for such coupler dispersion medium is preferred.

The use of high boiling point organic solvents which can be represented by the general formulae (A) to (E) indicated below is preferred.

In these formulae, W₁, W₂ and W₃ each represents a substituted or unsubstituted alkyl group, cycloalkyl group, alkenyl group, aryl group or heterocyclic group, W₄ represents W₁, OW₁ or S-W₁, and n represents an integer of from 1 to 5, and when n is 2 or more the W₄ groups may be the same or different. Moreover, W₁ and W₂ in general formula (E) may form a condensed ring.

Water immiscible compounds of having melting point of 100°C or lower and of boiling point or 140°C or higher other than those of general formulae (A) to (E) can also be used as high boiling point organic solvents in the present invention provided that they are good solvents for the coupler. The melting point of the high boiling point organic solvent is preferably not more than 80°C. Moreover, the boiling point of the high boiling point organic solvent is preferably at least 160°C, and most desirably at least 170°C.

Details of these high boiling point organic solvents have been disclosed from the lower right column on page 137 to the upper right column on page 144 in JP-A-62-215272.

Furthermore, these couplers can be loaded onto a loadable latex polymer (for example, U.S. Patent 4,203,716) in the presence or absence of the aforementioned high boiling point organic solvents, or they can be dissolved in a water insoluble but organic solvent soluble polymer and the solution can be emulsified and dispersed in an aqueous hydrophilic colloid solution.

The use of the homopolymers or copolymers disclosed on pages 12-30 of International Patent WO88/00723 is preferred, and the use of acrylamide based polymers is especially desirable from the viewpoint of colored image stabilization, etc.

The hydrophobic additive other than couplers is contained in the silver halide emulsion of the present invention in an amount of from 1x10⁻⁴ to 1.0 mol per mol of silver halide, and in a non-light sensitive layer of the present invention in an amount of from 1x10⁻⁴ to 1.0 g/m².

Light sensitive materials which is prepared using the present invention may contain hydroquinone derivatives, aminophenol derivatives, gallic acid derivatives and ascorbic acid derivatives, for example, as anti-color fogging agents.

Various anti-color fading agents can be used in light sensitive materials of the present invention. That is to say, hydroquinones, 6-hydroxychromans, 5-hydroxycoumarans, spirochromans, p-alkoxyphenols, bisphenols such as hindered phenols, gallic acid derivatives, methylenedioxybenzenes, aminophenols, hindered amines, and the ether and ester derivatives in which the phenolic hydroxyl groups of these compounds is silylated or alkylated, are typical organic anti-color mixing agents which can be used for cyan, magenta and/or yellow images. Furthermore, metal complexes as typified by (bis-salicylaldoximato)nickel and (bis-N,N-dialkyldithiocarbamato)nickel complexes, for example, can also be used for this purpose.

Examples of organic anti-color fading agents have been disclosed in patents indicated below.

Thus, hydroquinones are disclosed, for example, in U.S. Patents 2,360,290, 2,418,613, 2,700,453, 2,701,197, 2,728,659, 2,732,300, 2,735,765, 3,982,944 and 4,430,425, British Patent 1,363,921, and U.S. Patents 2,710,801 and 2,816,028, 6-hydroxychromans, 5-hydroxychromans and spirochromans are disclosed, for example, in U.S. Patents 3,432,300, 3,573,050, 3,574,627, 3,698,909 and 3,764,337, and JP-A-52-152225, spiroindanes are disclosed in U.S. Patent 4,360,589, p-alkoxyphenols are disclosed, for example, in U.S. Patent 2,735,765, British Patent 2,066,975, JP-A-59-10539 and JP-B-57-19765, hindered phenols are disclosed, for example, in U.S. Patent 3,700,455, JP-A-52-72224, U.S. Patent 4,228,235, and JP-B-52-6623, gallic acid derivatives, methylenedioxybenzenes and aminophenols are disclosed, for example, in U.S. Patents 3,457,079 and 4,332,886, and JP-B-56-21144, hindered amines are disclosed, for example, in U.S. Patents 3,336,135 and 4,268,593, British Patents 1,326,889, 1,354,313 and 1,410,846, JP-B-51 1420, JP-A-58-114036, JP-A-59-53846 and JP-A-59-78344, and metal complexes have been disclosed, for example, U.S. Patents 4,050,938 and 4,241,155, and British Patent 2,027,731(A). (The term "JP-B" as used herein signifies an "examined Japanese patent publication".) The intended purpose can be attained by adding these compounds to the photosensitive layer after co-emulsification with the corresponding color coupler, usually in an amount of from 5 to 100 wt% with respect to the coupler. The inclusion of ultraviolet absorbers in the cyan color forming layer and in the layers on both sides adjacent thereto is effective for preventing deterioration of the cyan dye image by heat and, more especially, by light.

For example, benzotriazole compounds substituted with aryl groups (for example, those disclosed in U.S. Patent 3,533,794), 4-thiazolidone compounds (for example, those disclosed in U.S. Patents 3,314,794 and 3,352,681), benzophenone compounds (for example, those disclosed in JP-A-46-2784), cinnamic acid ester compounds (for example, those disclosed in U.S. Patents 3,705,805 and 3,707,395), butadiene compounds (for example, those disclosed in U.S. Patent 4,045,229), or benzoxidol compounds (for example, those disclosed in U.S. Patents 3,406,070, 3,677,672 and 4,271,307) can be used as ultraviolet absorbers. Ultraviolet absorbing couplers (for example, α-naphthol based cyan dye forming couplers) and ultraviolet absorbing polymers, for example, can also be used for this purpose. These ultraviolet absorbers may be mordanted in a specified layer.

For among these compounds, the aforementioned benzotriazole compounds which are substituted with aryl groups are preferred.

The use, together with the couplers described above, of compounds such as those described below is preferred in the present invention. The cojoint use of these compounds with pyrazoloazole couplers is especially desirable.

Thus, the use of compounds (F) which chemically bond with the aromatic amine developing agents remaining after color development processing and form compounds which are chemically inert and essentially colorless and/or compounds (G) which chemically bond with the oxidized product of the aromatic amine color developing agents remaining after color development processing and form compounds which are chemically inert and essentially colorless, either in combination or individually, is desirable for preventing the occurrence of staining and other side effects on storage due to colored dye formation resulting from reactions between couplers and color developing agents or oxidized products thereof which remain in the film after processing for example.

Compounds which react with p-anisidine with a second order reaction rate constant k₂ (measured in trioctyl phosphate at 80°C) within the range from 1.0 liter/mol·sec to 1×10⁻⁵ liter/mol·sec are preferred for the compound (F). The second order reaction rate constant can be measured using the method disclosed in JP-A-63-158545.

The compounds themselves are unstable if k₂ has a value above this range, and they will react with gelatin or water and be decomposed. If, on the other hand, the value of k₂ is below this range, reaction with the residual aromatic amine developing agent is slow and consequently it is not possible to prevent the occurrence of side effects due to the residual aromatic amine developing agent.

The preferred compounds (F) of this type can be represented by the general formulae (FI) and (FII) which are shown below.
R₁-(A)ₙ-X (FI)
R₂- =Y (FII)

In these formulae, R₁ and R₂ each represent an aliphatic group, an aromatic group or a heterocyclic group. Moreover, n represents 1 or 0. A represents a group which reacts with an aromatic amine developing agent and forms a chemical bond, and X represents a group which is eliminated by reaction with an aromatic amine developing agent. B represents a hydrogen atom, an aliphatic group, an aromatic group, a heterocyclic group, an acyl group or a sulfonyl group, and Y represents a group which promotes the addition of an aromatic amine developing agent to the compound of general formula (FII). Here, R₁ and X, and Y and R₂ or B, can be joined together to form a cyclic structure.

Substitution reactions and addition reactions are typical of the reactions by which residual aromatic amine developing agents are chemically bound.

The actual examples of compounds represented by the general formulae (FI) and (FII) disclosed, for example, in JP-A 63-158545, JP-A-62-283338, and European Patents (laid open) 298,321 and 277,589 are preferred.

On the other hand, the preferred compounds (G) which bond chemically with the oxidized products of aromatic amine developing agents which remain after color development processing and form compounds which are chemically inert and colorless can be represented by the general formula (GI) indicated below.
R-Z (GI)

R in this formula represents an aliphatic group, an aromatic group or a heterocyclic group. Z represents a nucleophilic group or a group which breaks down in the light sensitive material and releases a nucleophilic group. The compounds represented by the general formula (GI) are preferably compounds in which Z is a group of which the Pearson nucleophilicity ⁿCH₃I value (R.G. Pearson et al., J. Am. Chem. Soc., 90, 319 (1968)) is at least 5, or a group derived therefrom.

The actual examples of compounds which can be represented by general formula (GI) disclosed, for example, in European Patent laid open 255,722, JP-A-62-143048, JP-A-62-229145, JP-A-1-57259, Japanese Patent Application No. 63-136724, and European Patents (laid open) 298,321 and 277,589 are preferred.

Furthermore, details of combinations of the aforementioned compounds (G) and compounds (F) have been disclosed in European Patent Laid Open No. 277,589.

Water soluble dyes and dyes which become water soluble as a result of photographic processing may be included as filter dyes, or for antiirradiation or antihalation or other purposes, in the hydrophilic colloid layers of light sensitive materials which is prepared using the present invention. Dyes of this type include oxonol dyes, hemi-oxonol dyes, styryl dyes, merocyanine dyes, cyanine dyes and azo dyes. The oxonol dyes, hemi- oxonol dyes and merocyanine dyes are useful among these dyes.

Gelatin is useful as a binding agent or protective colloid which can be used in the emulsion layers of light sensitive materials of the present invention, but other hydrophilic colloids, either alone or in combination with gelatin, can be used for this purpose.

The gelatin used in the invention may be a lime treated gelatin, or it may be acid treated gelatin. Details of the preparation of gelatins have been disclosed by Arthur Weise in The Macromolecular Chemistry of Gelatin (published by Academic Press, 1964).

The transparent films, such as cellulose nitrate films and poly(ethylene terephthalate) films, and reflective supports normally used in photographic light sensitive materials can be used as the supports which are used in thfe present invention. The use of reflective supports is preferred in view of the aims of the invention.

The "reflective supports" used in this present invention are supports which have a high reflectivity and make the dye image which is formed in the silver halide emulsion layer clear, and they include supports which are covered with a hydrophobic resin containing a dispersion of light reflecting material, such as titanium oxide, zinc oxide, calcium carbonate or calcium sulfate, and supports comprised of a hydrophobic resin in which contains a dispersion of a light reflecting substance. Examples of such supports include baryta paper, polyethylene coated paper, polypropylene based synthetic paper and transparent supports, such as glass plates, polyester films such as poly(ethylene terephthalate), cellulose triacetate and cellulose nitrate films, polyamide films, polycarbonate films, polystyrene films and vinyl chloride resins, on which a reflective layer is provided or in which a reflective substance is used conjointly.

Supports which have a metal surface with mirror like reflection properties or a type secondary diffuse reflective metal surface can be used as reflective type supports. The spectral reflectance in the visible wavelength region of the metal surface is at least 0.5, and diffuse reflection properties can be attained by roughening the metal surface, or by using a metal powder. Aluminum, tin, silver, magnesium or their alloys are used, for example, as the metal, and the surface may be a metal sheet, a metal foil or a thin metal layer obtained by rolling, vapor deposition or plating for example. From among these materials, those obtained by vapor depositing metal on some other substrate are preferred. It is preferrred to provide a water insoluble resin layer, preferably a thermoplastic resin layer over the metal surface. An anti-static layer may also be provided on the opposite side to the metal surface side of the support in the preesnt invention. Details of such supports is disclosed, for example, in JP-A-61-210346, JP-A-63-24247, JP-A-63-24251 and JP A-63-24255.

These supports can be selected appropriately according to the intended use.

### EXAMPLE 1 (Blue Sensitive Layer)

Ethyl acetate (27.2 ml) and 8.2 grams of solvent (Solv-1) were added to 19.1 grams of yellow coupler (ExY), 4.4 grams of color image stabilizer (Cpd-1) and 0.7 gram of color image stabilizer (Cpd-7), and the solution was emulsified and dispersed in 185 ml of 10% aqueous gelatin solution which contained 8 ml of 10% sodium dodecylbenzenesulfonate. The average particle size of the emulsified dispersion was 0.12 µm. On the other hand, the blue sensitive sensitizing dyes indicated below were added in an amount of 2.0×10⁻⁴ mol per mol of silver for the large size emulsion and 2.5×10⁻⁴ mol per mol of silver halide for the small size emulsion to a silver chlorobromide emulsion (a 3:7 (mol ratio) mixture; cubic; average grain size: 0.88 µm and 0.70 µm; variation coefficients of the grain size distributions: 0.08 and 0.10; which contained locally 0.2 mol% of silver bromide on the grain surfaces), and sulfur sensitization was carried out. The aforementioned emulsified dispersion was mixed under the conditions indicated below with the emulsion which was prepared in the way described above to provide the coating liquids (a), (b), (c) and (d) indicated below.

| Coating Liquid | Storage Time of the Emulsified Dispersion Before Preparing the Coating Liquid | Storage Temp. of the Emulsified Dispersion | Remarks |
|---|---|---|---|
| (a) | 6 hrs | 35°C | Invention |
| (b) | 24 hrs | 35°C | " |
| (c) | 48 hrs | 35°C | Comp. Ex. |
| (d) | 72 hrs | 35°C | " |

These coating liquids and a gelatin protective layer coating liquid as an over-layer were coated onto paper supports which had been laminated on both sides with polyethylene to obtain single layer color printing paper samples 101, 102, 103 and 104. The average standing time of each coating liquid was 3 hours. .

1-Oxy-3,5-dichloro-s-triazine sodium salt was used as a gelatin hardening agent.

The following dyes were used as the spectrally sensitizing dyes: (2.0×10⁻⁴ mol per mol of silver halide in the large size emulsion, and 2.5×10⁻⁴ mol per mol of silver halide in the small size emulsion)

Furthermore, 1-(5-methylureidophenyl)-5-mercaptotetrazole was added in an amount of 8.5×10⁻⁵ mol per mol of silver halide.

### Layer Structure

The composition of each layer was as indicated below. The numerical values indicate coated weights (g/m²). The coated weights of silver halide emulsion are indicated as calculated coated silver weights.
Support
Polyethylene Laminated Paper
[White pigment (TiO₂) in the polyethylene on the first layer side]

| First Layer: Blue Sensitive Layer | |
|---|---|
| The aforementioned silver chlorobromide emulsion | 0.30 |
| Gelatin | 1.86 |
| Yellow coupler (ExY) | 0.82 |
| Color image stabilizer (Cpd-1) | 0.19 |
| Solvent (Solv-1) | 0.35 |
| Color image stabilizer (Cpd-7) | 0.06 |

| Second Layer: Protective Layer | |
|---|---|
| Gelatin | 1.33 |
| Acrylic modified copolymer of poly(vinyl alcohol) (17% modification) | 0.17 |
| Liquid paraffin | 0.03 |

The following tests were carried out in order to investigate the photographic characteristics of these samples 101 to 104.

First of all, each sample was subjected to a gradation exposure using a sensitometer (FWH model, made by Fuji Photo Film Co., Ltd. light source color temperature 3200°K). The exposure at this time was 250 CMS with an exposure time of 0.1 second. The exposed samples were color developed using a paper processor in accordance with the processing operations indicated below.

| Procession Operation | Temperature | Time |
|---|---|---|
| Color Development | 35°C | 45 seconds |
| Bleach-fixing | 30-35°C | 45 seconds |
| Rinse (1) | 30-35°C | 20 seconds |
| Rinse (2) | 30-35°C | 20 seconds |
| Rinse (3) | 30-35°C | 20 seconds |
| Drying | 70-80°C | 60 seconds |
| (Three tank counter-flow system from Rinse (3) to Rinse (1)). | | |

The composition of each of the processing baths is indicated below.

| Color Development Bath | |
|---|---|
| Water | 800 mℓ |
| Ethylenediamine-N,N,N′,N′-tetramethylene phosphonic acid | 1.5 g |
| Potassium bromide | 0.015 g |
| Triethanolamine | 8.0 g |
| Sodium chloride | 1.4 g |
| Potassium carbonate | 25 g |
| | |
| N-Ethyl-N-(β-methanesulfonamidoethyl)-3-methyl-4-aminoaniline sulfate | 5.0 g |
| N,N-Bis(carboxymethyl)hydrazine | 5.5 g |
| Fluorescent whitener (Whitex 4B, made by Sumitomo Chemicals) | 1.0 g |
| Water | to make up to 1000 ml |
| pH (25°C) | 10.05 |

| Bleach-fix Bath | |
|---|---|
| Water | 400 ml |
| Ammonium thiosulfate (700 g/l aqueous solution) | 100 ml |
| Sodium sulfate | 17 g |
| Ethylenediamine tetraacetic acid iron(III) ammonium salt | 55 g |
| Ethylenediamine tetraacetic acid di-sodium salt | 5 g |
| Ammonium bromide | 40 g |
| Water | to make up to 1000 ml |
| pH (25°C) | 6.0 |

Rinse Bath
Ion exchanged water (calcium and magnesium both less than 3 ppm)

The yellow density of each developed sample was measured, and the survival rate of an initial density of 1.5 after 9 weeks irradiation with light of 17,000 lux was measured in order to evaluate the light fastness of the yellow image.

**Table 1**

| Sample | S_{0.5}* | Maximum Density (Dmax) | Survival Rate | Remarks |
|---|---|---|---|---|
| | | | (%) | |
| 101 | 1.10 | 2.40 | 87 | Invention |
| 102 | 1.10 | 2.38 | 85 | " |
| 103 | 1.08 | 2.32 | 82 | Comp. Ex. |
| 104 | 1.07 | 2.26 | 79 | " |

| | | | | |
|---|---|---|---|---|
| *S_{0.5}: value of log E at fog+density 0.5 | | | | |

It is clear from the results shown in Table 1 that samples 101 and 102 where the storage time of the emulsified dispersion was short had a higher photographic speed and a higher survival rate of an initial density of 1.5.

The fact that the sensitive materials of the present invention should have such a high photographic speed and such a large survival rate was completely unforeseen.

### EXAMPLE 2 (Green Sensitive Layer)

Ethyl acetate (27.2 ml) and 28.7 grams of solvent (Solv-2) were added to 14.14 grams of magenta coupler (EXM), 8.84 grams of color image stabilizer (Cpd-3), 1.33 grams of color image stabilizer (Cpd-8), 0.44 grams of color image stabilizer (Cpd-4) and 1.77 grams of color image stabilizer (Cpd-9) and the solution was emulsified and dispersed in 200 ml of 10% aqueous gelatin solution which contained 5.5 ml of 10% sodium dodecylbenzenesulfonate. The particle size immediately after emulsification was 0.15 µm.

On the other hand, the green sensitive sensitizing dyes indicated below were added to a silver chloride emulsion (a 1:3 (silver mol ratio) mixture of cubic silver halide grain emulsions of average grain size 0.55 µm and 0.39 µm, of which the variation coefficients of the grain size distributions were 0.10 and 0.08, respectively, which contained locally 0.8 mol% of silver bromide on the grain surfaces), and sulfur sensitization was carried out. The aforementioned emulsified dispersion was mixed under the conditions indicated below with the emulsion which was prepared in the way described above to provide the coating liquids 2-(a), 2-(b), 2-(c) and 2-(d) indicated below.

| Coating Liquid | Storage Time of the Emulsified Dispersion Before Preparing the Coating Liquid | Storage Temp. of the Emulsified Dispersion | Remarks |
|---|---|---|---|
| 2-(a) | 6 hrs | 40°C | Invention |
| 2-(b) | 24 hrs | 40°C | " |
| 2-(c) | 48 hrs | 40°C | Comp. Ex. |
| 2-(d) | 72 hrs | 40°C | " |

These coating liquids and a gelatin protective layer coating liquid as an over-layer were coated onto paper supports which had been laminated on both sides with polyethylene to obtain single layer color printing paper samples 201, 202, 203 and 204. The average standing time of each coating liquid was three hours.

1-Oxy-3,5-dichloro-s-triazine sodium salt was used as a gelatin hardening agent.

The following dyes were used for the spectrally sensitizing dyes: (4.0×10⁻⁴ per mol of silver halide in the large size emulsion, 5.6×10⁻⁴ mol per mol of silver halide in the small size emulsion) and: (7.0×10⁻⁵ mol per mol of silver halide in the large size emulsion, and 1.0×10⁻⁵ mol per mol of silver halide in the small size emulsion)

Furthermore, 1-(5-methylureidophenyl)-5-mercaptotetrazole was added in an amount of 7.7×10⁻⁴ mol per mol of silver halide, respectively.

### Layer Structure

The composition of each layer was as indicated below. The numerical values indicate coated weights (g/m²). The coated weights of silver halide emulsion are indicated as calculated coated silver weights.
Support
Polyethylene Laminated Paper
[White pigment (TiO₂) in the polyethylene on the first layer side]

| First Layer: Blue Sensitive Layer | |
|---|---|
| The aforementioned silver chlorobromide emulsion | 0.12 |
| Gelatin | 1.24 |
| Magenta coupler (ExM) | 0.20 |
| Color image stabilizer (Cpd-2) | 0.03 |
| Color image stabilizer (Cpd-3) | 0.15 |
| Color image stabilizer (Cpd-4) | 0.02 |
| Color image stabilizer (Cpd-9) | 0.02 |
| Solvent (Solv-2) | 0.40 |

Second Layer: Protective Layer
Same as in Example 1

These samples were exposed and developed in the same way as described in Example 1, the magenta densities were measured, and the light fastness was evaluated using the same method as described in Example 1. The results obtained are shown in Table 2.

**Table 2**

| Sample | S_{0.5} | Maximum Density (Dmax) | Survival Rate | Remarks |
|---|---|---|---|---|
| | | | (%) | |
| 201 | 1.20 | 2.62 | 87 | Invention |
| 202 | 1.20 | 2.58 | 85 | " |
| 203 | 1.19 | 2.48 | 82 | Comp. Ex. |
| 204 | 1.18 | 2.40 | 77 | " |

It is clear from the results shown in Table 2 that samples 201 and 202 where the storage time of the emulsified dispersion was short had a higher photographic speed and a higher survival rate of an initial density of 1.5.

The fact that the sensitive materials of this present invention should have such a high photographic speed and such a large survival rate was completely unforeseen.

### EXAMPLE 3 (Red Sensitive Layer)

Ethyl acetate (23 ml) and 7.5 grams of solvent (Solv-6) were added to 16 grams of cyan coupler (ExC), 8.5 grams of color image stabilizer (Cpd-6), 20 grams of color image stabilizer (Cpd-7), 2 grams of color image stabilizer (Cpd-8) and the solution was emulsified and dispersed in 140 ml of 10% aqueous gelatin solution which contained 10 ml of 10% sodium dodecylbenzenesulfonate. The particle size immediately after emulsification was 0.08 µm. On the other hand, the red sensitive sensitizing dye indicated below was added in an amount of 0.9×10⁻⁴ mol of per mol of silver for the large size emulsion and 1.1×10⁻⁴ mol per mol of silver halide for the small size emulsion to a silver chlorobromide emulsion (a 1:4 (silver mol ratio) mixture of cubic silver halide grain emulsions of average grain size 0.58 µm and 0.45 µm, of which the variation coefficients of the grain size distributions were 0.09 and 0.11, respectively, and which contained locally 0.6 mol% of silver bromide on the grain surfaces), and sulfur sensitization was carried out. The aforementioned emulsified dispersion was mixed under the conditions indicated below with the emulsion which had been prepared in the way described above to provide the coating liquids 3-(a), 3-(b), 3-(c) and 3-(d) indicated below.

| Coating Liquid | Storage Time of the Emulsified Dispersion Before Preparing the Coating Liquid | Storage Temp. of the Emulsified Dispersion | Remarks |
|---|---|---|---|
| 3-(a) | 6 hrs | 40°C | Invention |
| 3-(b) | 24 hrs | 40°C | " |
| 3-(c) | 48 hrs | 40°C | Comp. Ex. |
| 3-(d) | 72 hrs | 40°C | " |

These coating liquids and a gelatin protective layer coating liquid as an over-layer were coated onto paper supports which had been laminated on both sides with polyethylene to obtain single layer color printing papers samples 301, 302, 303 and 304. The average standing time of each coating liquid was three hours.

1-Oxy-3,5-dichloro-s-triazine sodium salt was used as a gelatin hardening agent.

The following dyes were used for the spectrally sensitizing dyes: (0.9×10⁻⁴ mol per mol of silver halide in the large size emulsion, 1.1×10⁻⁴ mol per mol of silver halide in the small size emulsion)

Furthermore, the compound indicated below was added in an amount of 2.6×10⁻³ mol per mol of silver halide.

Furthermore, 1-(5-methylureidophenyl)-5-mercaptotetrazole was added in an amount of 2.5×10⁻⁴ mol per mol of silver halide, respectively.

### Layer Structure

The composition of each layer was as indicated below. The numerical values indicate coated weights (g/m²). The coated weights of silver halide emulsion are indicated as calculated coated silver weights.
Support
Polyethylene Laminated Paper
[White pigment (TiO₂) in the polyethylene on the first layer side]

| First Layer: Red Sensitive Layer | |
|---|---|
| The aforementioned silver chlorobromide emulsion | 0.23 |
| Gelatin | 1.34 |
| Cyan coupler (ExC) | 0.32 |
| Color image stabilizer (Cpd-6) | 0.17 |
| Color image stabilizer (Cpd-7) | 0.40 |
| Color image stabilizer (Cpd-8) | 0.04 |
| Solvent (Solv-6) | 0.15 |

Second Layer: Protective Layer
Same as in Example 1

These samples were exposed and developed in the same way as described in Example 1, the magenta densities were measured, and the light fastness was evaluated using the same method as described in Example 1. The results obtained are shown in Table 3.

**Table 3**

| Sample | S_{0.5} | Maximum Density (Dmax) | Survival Rate | Remarks |
|---|---|---|---|---|
| | | | (%) | |
| 301 | 1.16 | 2.80 | 89 | Invention |
| 302 | 1.15 | 2.76 | 88 | " |
| 303 | 1.13 | 2.66 | 84 | Comp. Ex. |
| 304 | 1.11 | 2.58 | 80 | " |

It is clear from the results shown in Table 2 that samples 301 and 302 where the storage time of the emulsified dispersion was short had a higher photogra phic speed and a higher survival rate of an initial density of 1.5.

The fact that the sensitive materials of this present invention should have such a high photographic speed and such a large survival rate was completely unforeseen.

### EXAMPLE 4 (Blue Sensitive Layer and UV Absorbing Non-photosensitive layer

Ethyl acetate (5.4 ml) and 5.1 grams of solvent (Solv-5) were added to 10.2 gram of ultraviolet absorber (UV-1) and 1.3 grams of anti-color mixing agent (Cpd-5) and the solution was emulsified and dispersed in 140 ml of 10% aqueous gelatin solution which contained 10 ml of 10% sodium dodecylbenzenesulfonate. The particle size immediately after emulsification was 0.05 µm.

This emulsified dispersion was mixed with 15% aqueous gelatin solution to provide the coating liquids 4-(a), 4-(b), 4-(c) and 4-(d).

| Coating Liquid | Storage Time of the Emulsified Dispersion Before Preparing the Coating Liquid | Storage Temp. of the Emulsified Dispersion | Remarks |
|---|---|---|---|
| 4-(a) | 6 hrs | 40°C | Invention |
| 4-(b) | 24 hrs | 40°C | " |
| 4-(c) | 48 hrs | 40°C | Comp. Ex. |
| 4-(d) | 72 hrs | 40°C | " |

These coating liquids, the coating liquid (a) described in Example 1 as an under-layer and the protective layer coating liquid described in Example 1 as an over-layer were coated onto paper supports which had been laminated on both sides with polyethylene to obtain single layer color printing paper samples 401, 402, 403 and 404, respectively. The average standing times of the coating liquids were 3 hours.

1-Oxy-3,5-dichloro-s-triazine sodium salt was used as a gelatin hardening agent.

These samples were exposed and developed in the same way as described in Example 1 and the light fastness of the yellow dye was evaluated using the same method as described in Example 1. The results obtained are shown in Table 4.

**Table 4**

| Sample | Survival | Staining (Minimum Yellow Density) | Remarks |
|---|---|---|---|
| | (%) | | |
| 401 | 87 | 0.28 | Invention |
| 402 | 87 | 0.28 | " |
| 403 | 87 | 0.30 | Comp. Ex. |
| 404 | 86 | 0.31 | " |

It is clear from the results shown in Table 4 that samples 401 and 402 where the storage time of the emulsified dispersion was short were less liable to staining.

This effect was completely unforeseen.

### EXAMPLE 5 (All Layers)

Multi-layer color printing paper samples 501 to 506 of which the layer structure is indicated below, were prepared using coating liquid (a) of Example 1, coating liquid 2-(a) of Example 2, coating liquid 3-(a) of Example 3 and coating liquid 4-(a) of Example 4 under the conditions indicated below on paper supports which had been laminated on both sides with polyethylene.

1-Oxy-3,5-dichloro-s-triazine sodium salt was used as a gelatin hardening agent in each layer.

The dyes indicated below were added to the emulsion layers for anti-irradiation purposes.

### Layer Structure

The composition of each layer was as indicated below. The numerical values indicate coated weights (g/m²). The coated weights of silver halide emulsion are indicated as calculated coated silver weights.
Support
Polyethylene Laminated Paper
[White pigment (TiO₂) in the polyethylene on the first layer side]
First Layer: Blue Sensitive Layer

Same as in Example 1.

| Second Layer: Anti-color Mixing Layer | |
|---|---|
| Gelatin | 0.99 |
| Anti-color mixing agent (Cpd-5) | 0.08 |
| Solvent (Solv-1) | 0.16 |
| Solvent (Solv-4) | 0.08 |

Third Layer: Green Sensitive Layer

Same as in Example 2

| Fourth Layer: Ultraviolet Absorbing Layer | |
|---|---|
| Gelatin | 1.58 |
| Ultraviolet absorber (UV-1) | 0.47 |
| Anti-color mixing agent (Cpd-5) | 0.05 |
| Solvent (Solv-5) | 0.24 |

Fifth Layer: Red Sensitive Layer

Same as in Example 3

| Sixth Layer: Ultraviolet Absorbing Layer | |
|---|---|
| Gelatin | 0.53 |
| Ultraviolet absorber (UV-1) | |
| Anti-color mixing agent (Cpd-5) | |
| Solvent (Solv-5) | |

Seventh Layer: Protective Layer
Same as in Example 1

| | Coating Liquid Standing Time | | | |
|---|---|---|---|---|
| Sample | Blue Sensitive Layer | Green Sensitive Layer | Red Sensitive Layer | Remarks |
| | (min.) | (min.) | (min.) | |
| 501 | 10 | 10 | 10 | Invention |
| 502 | 30 | 30 | 30 | " |
| 503 | 60 | 60 | 60 | " |
| 504 | 120 | 120 | 120 | " |
| 505 | 180 | 180 | 180 | " |
| 506 | 240 | 240 | 240 | Comp. Ex. |

The tests indicated below were carried out in order to investigate the photographic characteristics of these samples.

First of all, each sample was subjected to a gradation exposure using a sensitometer (FWH model, made by the Fuji Photo Film Co., Ltd. light source color temperature 3200°K) with sensitometric tri-color (blue, green and red) separation filters. The exposure at this time was 250 CMS with an exposure time of 0.1 second.

The exposed samples were developed and processed using the method described in Example 1.

The yellow, magenta and cyan images densities of each developed sample were measured. The results obtained are shown in Table 5.

**Table 5**

| | Photographic Speed | | | Maximum Density | | | |
|---|---|---|---|---|---|---|---|
| Sample | Blue Sensitive Layer | Green Sensitive Layer | Red Sensitive Layer | Blue Sensitive Layer | Green Sensitive Layer | Red Sensitive Layer | Remarks |
| 501 | 1.10 | 1.20 | 1.16 | 2.40 | 2.62 | 2.80 | Invention |
| 502 | 1.10 | 1.20 | 1.15 | 2.40 | 2.62 | 2.80 | " |
| 503 | 1.10 | 1.20 | 1.16 | 2.39 | 2.60 | 2.80 | " |
| 504 | 1.10 | 1.20 | 1.16 | 2.39 | 2.60 | 2.78 | " |
| 505 | 1.09 | 1.19 | 1.14 | 2.35 | 2.57 | 2.73 | " |
| 506 | 1.09 | 1.19 | 1.10 | 2.31 | 2.55 | 2.65 | Comp. Ex. |

It is clear from the results shown in Table 5 that Samples 501 to 505 of this invention where the coating liquids were coated within 3 hours had a high speed and provided higher maximum densities, and this effect was especially pronounced with Samples 501 to 503 which were coated within 1 hour, and it is more pronounced with Samples 501 and 502 which were coated within 30 minutes.

### EFFECT OF THE INVENTION

Color photographic photosensitive materials which are manufactured in accordance with the present invention have a high photographic speed and a high maximum density, and they also provide color photographs which have excellent fastness. Furthermore, the invention is also effective in that staining in non-colored parts is suppressed. Furthermore, coating troubles can be prevented by the application of this present invention.

While the invention has been described in detail and with reference to specific embodiments thereof, it will be apparent to one skilled in the art that various changes and modifications can be made therein without departing from the spirit and scope thereof.

## Claims

1. A method for manufacturing a silver halide color photographic light sensitive material comprising a support having thereon at least one of light sensitive silver halide emulsion layer and non-light sensitive hydrophilic colloid layer which contains at least one hydrophobic photographically useful additive, which comprises preparing a hydrophilic colloid emulsified dispersion of said hydrophobic photographically useful additive, mixing the emulsified dispersion within 24 hours with the remaining coating composition of the layer and coating the mixture obtained on the support.

2. A method for manufacturing a silver halide color photographic light sensitive material as in claim 1, wherein the mixture of the hydrophilic colloid emulsified dispersion and the remaining coating composition is coated within three hours after mixing.

3. A method for manufacturing a silver halide color photographic light sensitive material as in claim 1, wherein said at least one hydrophobic photographically useful additive is at least one compound selected from the group consisting of couplers, anti-color mixing agents, antifoggants, anti-color fading agents, antistaining agents, ultraviolet absorbers, and slidability improving agents.

4. A method for manufacturing a silver halide color photographic light sensitive material as in claim 1, wherein the hydrophilic colloid is gelatin.

5. A method for manufacturing a silver halide color photographic light sensitive material as in claim 1, wherein said hydrophilic colloid emulsified dispersion is provided by dispersing said at least one hydrophobic photographically useful additive into a hydrophilic colloid aqueous solution containing a surfactant.

6. A method for manufacturing a silver halide color photographic light sensitive material as in claim 1, wherein said hydrophilic colloid aqueous solution is a 10 to 50% gelatin aqueous solution.

7. A method for manufacturing a silver halide color photographic light sensitive material as in claim 1, wherein said at least one hydrophobic photographically useful additive is dispersed in a hydrophilic colloid aqueous solution as an organic solvent solution thereof.

8. A method for manufacturing a silver halide color photographic light sensitive material as in claim 7, wherein said solution contains said at least one hydrophobic photographically useful additive in an amount of from 50 to 150% by weight based on the weight of the solvent.

9. A method for manufacturing a silver halide color photographic light sensitive material as in claim 7, wherein the organic solvent of the solution comprises a high boiling point organic solvent.

10. A method for manufacturing a silver halide color photographic light sensitive material as in claim 7, wherein the organic solvent of the solution comprises a high boiling point organic solvent in an amount of up to 10 weight% based on the total weight of the dispersion.

11. method for manufacturing a silver halide color photographic light sensitive material as in claim 7, wherein the solvent of the solution is a low boiling point organic solvent which is removed from the coating composition prior to mixing.

12. A method for manufacturing a silver halide color photographic light sensitive material as in claim 1, wherein the layer containing at least one hydrophobic photographically useful additive is a light sensitive silver halide emulsion layer and the remaining coating composition is a light sensitive silver halide emulsion.

13. A method for manufacturing a silver halide color photographic light sensitive material as in claim 12, wherein said hydrophobic photographically useful additive is at least one coupler.

14. A method for manufacturing a silver halide color photographic light sensitive material as in claim 12, wherein said hydrophobic photographically useful additive is at least one cyan coupler.

15. A method for manufacturing a silver halide color photographic light sensitive material as in claim 12, wherein said light sensitive silver halide emulsion contains at least one sensitizing dye.

16. A method for manufacturing a silver halide color photographic light sensitive material as in claim 1, wherein the layer containing at least one hydrophobic photographically useful additive is a non-light sensitive hydrophilic colloid layer.

17. A method for manufacturing a silver halide color photographic light sensitive material as in claim 16, wherein said non-light sensitive hydrophilic colloid layer is a protective layer, an intermediate layer or an antihalation layer.

18. A method for manufacturing a silver halide color photographic light sensitive material as in claim 16, wherein said at least one hydrophobic photographically useful additive is an ultraviolet absorber.

19. A method for manufacturing a silver halide color photographic light sensitive material as in claim 2, wherein said hydrophobic photographically useful additive is dispersed in the mixture as drops having an average particle size of not more than 0.2 µm.

20. A method for manufacturing a silver halide color photographic light sensitive material as in claim 1, wherein the amount of the hydrophilic colloid emulsified dispersion is from 1 to 70% by weight based on the total weight of the coating composition obtained by mixing the dispersion with the remained coating composition.

21. A method for manufacturing a silver halide color photographic light sensitive material as in claim 20, wherein the amount of the hydrophilic colloid emulsified dispersion containing a liquid paraffin as a photographically useful agent is from 1 to 10% by weight based on the total weight of the coating composition obtained by mixing the dispersion with the remained coating composition.

22. A method for manufacturing a silver halide color photographic light sensitive material as in claim 1, wherein said at least one light sensitive silver halide emulsion contains silver chlorobromide or silver chloride.
